

2,047,773

July 14, 1936.

E. W. GREENE ET AL  
ORE CONCENTRATING MACHINE

Filed Oct. 31, 1934



FIG. 3.



FIG. 4.



FIG. 5.



INVENTOR  
E. W. Greene  
R. M. Wilbur  
BY Arthur H. Sennell  
their ATTORNEY

## UNITED STATES PATENT OFFICE

2,047,773

## ORE CONCENTRATING MACHINE

Ernest W. Greene and Robert M. Wilbur, Plant  
City, Fla., assignors to Coronet Phosphate  
Company, New York, N. Y., a corporation of  
New York

Application October 31, 1934, Serial No. 750,787

9 Claims. (Cl. 209—431)

Our invention pertains to a machine for ore concentration. Prior to the present invention the concentration of finely divided ores, by means of flotation, was mainly accomplished by aerating and agitating a chemically treated pulp of the ore under water. Such a process is generally referred to in the art as a froth flotation process and is carried out in a froth flotation machine. In this well-known type of apparatus it is customary to provide mechanical agitation in order to maintain the ore in suspension in the flotation vessels. The floatable constituent of the ore attaches itself to the air bubbles and is thus raised to the surface of the water. A stable froth supports the ore on the water surface and permits it to be floated off.

In accordance with the teaching of the present invention a thick pulp of chemically treated ore is fed continuously on to a moving belt. Water is supplied to the belt so as to maintain a flow over both sides. Baffle elements drag on the surface of the belt to prevent the non-floatable portion of the ore from being washed off the sides, and serve to plow up or turn over the pile of ore on the belt. The plowing action thus obtained continually presents fresh parts of the ore pile to the water surface for flotation. The floatable constituent of the ore floats or is washed off the sides of the belt and is caught in suitable launders. The non-floatable constituent of the ore remains on the belt and is finally carried off the end by the movement of the belt.

Certain advantages of the invention over previous practice in the art are due principally to the fact that the ore is maintained at, or near, the water surface at all times. Aerating and agitating in the sense used in froth flotation machines have been eliminated. A froth is not maintained on the surface of the water. Since the elevation of the floatable constituent to the water surface does not depend on air bubbles, larger particles can be floated. Thus the usual grinding and classifying operations are not necessary. The separating action of the belt apparatus constructed in accordance with the present inventive conception is more efficient than that of the sub-aeration, froth flotation machine, because the floatable constituent of the ore is not raised through any appreciable depth of water, and is mechanically moved into the water surface. The side edges of the belt, off which the concentrates flow, are as low as, or lower than, the ore on the belt.

Our invention further includes other advantages and novel features of design, construction

and arrangement, hereinafter more particularly referred to in connection with the accompanying drawing in which Fig. 1 is an isometric view of the essential parts of the machine, assembled in their relative positions to each other. For purposes of clarity the supporting structure has not been included.

Figure 2 is a sectional view of the machine taken on line A—A, and

Figures 3, 4 and 5 are isometric views of the individual types of baffles employed in connection with the apparatus.

Referring to the drawing, a continuous belt is indicated at 1, which is preferably a type similar to the ordinary rubber conveyor belt. The width and the length of the belt may be suited to the tonnage and conditions desired from the machine. In general, larger tonnages can be handled with wider and longer belts. Tonnages up to 30 tons per hour of feed have been handled successfully on a belt which was 30 inches wide and 50 feet long between pulleys. The belt 1 operates on pulleys indicated in the drawing at 2. The bearings for the belt pulleys 2, the supporting structure for the bearings, and the drive mechanism for the belt are not shown, and may be similar to those used in any conveyor belt installation. The belt may be driven at any linear speed up to about 100 feet per minute, depending on the tonnage and the conditions desired. The direction of motion of the belt is indicated by the arrow. The belt is maintained in a flat, level position by a number of longitudinal support members shown at 12 in Fig. 2 of the drawing.

The belt is fed with a fairly thick pulp of chemically treated ore fines through a feed chute 3 located at one end of the machine. The belt and the material on it are watered from above by means of jets extending along the under surfaces of the longitudinally located overhead pipes indicated in the drawing at 4.

Baffle members are indicated in the drawing at 5, 6 and 7, the same dragging on the side surface of the belt 1, being positioned, with respect to the belt, by means of longitudinally extending stationary pieces 8, which are provided with holes to receive the ends of the baffles. The individual types of baffles herein employed are indicated in detail in Figs. 3, 4 and 5 and the arrangement of the same in Fig. 1 is preferable when the machine is operating with a belt length of fifty feet.

The baffle 5 shown in Figure 3 is constructed by attaching a piece of sheet metal to a small bent metal rod. The sheet metal may be any metal of moderate thickness and adequate rigid-

ity. On a belt thirty inches wide, 20-28 gauge galvanized iron baffles which were  $2\frac{1}{2} \times 18$  inches have been used, although these specifications are not strictly required. The metal rod is preferably about  $\frac{1}{4}$  inch in diameter and may be any desirable material. Rust and corrosion resistant metals are preferable for these baffles. Baffles 6 and 7, shown in Figures 4 and 5, are bent rods, and the preceding description applies with equal effectiveness to their construction. The angle which the baffles 5, 6 and 7 make, with the direction of motion of the belt 1, vary considerably, angles of from  $20^\circ$  to  $45^\circ$  having been found to be most efficient in practical use. The baffles are angularly positioned with respect to the belt to direct the ore toward the central portion of the same during movement. The parallel arrangement of the baffles, which extends substantially along the entire side of the belt, further provides an unimpeded passageway along the same for the movement of the ore. In the construction illustrated, the baffles extend less than half way across the width of the belt.

The functions of these baffles are to turn over the pile of ore as it is moved past them by the belt and to prevent the non-floatable constituent being washed off the side edges of the belt. In the former respect their action is a plowing action which raises the ore above the water surface and then drops it into the water again. The latter effect is purely a baffle action. The baffles 5 in Figure 3 are more effective for keeping the non-floatable material on the belt, while the types 6 and 7 have a better turning action on the material. The arrangement of the baffles on the belt will depend on the conditions and the results desired. We have found that a desirable arrangement for a roughing operation is to equip the first half of the belt with type 5 baffles and the last half with types 6 and 7 baffles. We have found that a cleaning operation on medium grade concentrates works well with type 5 baffles on the whole length of the belt.

The spacing of the baffles along the belt depends on the width of the belt, the speed of the belt, the tonnage handled, and the grade of product taken off. We have found that a spacing of about 6 inches produces good results under quite a wide variation of conditions. The transversely level rigid baffles of the invention as illustrated are relatively closely spaced in parallel arrangement to extend substantially along the entire side surface of the belt. The position of the baffles along the side of the belt and only partially extending across the width of the same provides an area adjacent the inwardly disposed ends of the baffles for the free passage of ore along the belt.

The floatable constituent of the treated ore moves off the sides of the belt and is caught in a concentrate launder, shown at 9 in the drawing. The non-floatable constituent or tailing is carried along on the belt and over the end pulley where it is washed off with a tailing wash 10 into a tailing trough 11.

The separating action of the apparatus which has been described above is due to a combination of effects. The water jets from the pipes 4 penetrate the pile of ore, and on flowing out of, or off, the pile, this water carries a float concentrate on its surface. The plowing action of the baffles causes a float concentrate to form where the ore is moved out of, or into, the water on the belt. On flowing off of the belt the water washes with

it some coagulated material. There is never any appreciable depth of water maintained on the flat belt. The ore on the belt is thus always at, or near, the water surface.

The belt machine, which has been described above, would undoubtedly lend itself to the concentration of fine metalliferous and nonmetalliferous ores in general. The apparatus has been thoroughly tested on fine Florida phosphate ores. The belt used for this purpose was 30 inches wide and 50 feet between pulleys.

These tests were run with tailings from a screening concentration of Florida pebble phosphate rock. This material consisted principally of fine bone phosphate of lime and fine silica gangue which had passed a 0.032 inch screen and which had been deslimed. In all tests the deslimed phosphate fines were mixed with approximately the following amounts of reagents in pounds per ton of dry ore: 1 pound of solid caustic soda; 5 to 6 pounds of crude oil; 1 to 2 pounds of a crude mixture of fatty acids; 0 to 0.7 pounds of pine oil; sufficient water to give a freely flowing pulp.

The following examples have been taken from over 70 tests on the apparatus, and include two roughing tests and two cleaning tests. In the roughing tests low grade heads were fed to the apparatus, and medium grade concentrates and clean tailings were produced. In the cleaning tests medium grade material, which had been obtained as roughing concentrates, was fed to the apparatus without any further addition of reagents. These cleaning tests produced high grade concentrates and a middling.

*Example 1—(Roughing test).*—The first half of the belt was equipped with type 5 baffles and the last half with type 7 baffles. The linear speed of the belt was 38 feet per minute. A total of 600 pounds of chemically treated ore fines was fed to the watered belt at a rate of 15 long tons per hour. The results are recorded in the following table. "B. P. L." refers to bone phosphate of lime.

|            | Weights | B. P. L. | Recoveries | 45 |
|------------|---------|----------|------------|----|
|            | Percent | Percent  | Percent    |    |
| Heads..... | 100.0   | 37.36    | 100.0      |    |
| Concs..... | 52.6    | 66.70    | 93.9       |    |
| Tails..... | 47.4    | 4.80     | 6.1        | 50 |

*Example 2—(Roughing test).*—The first half of the belt was equipped with type 5 baffles and the last half with types 6 and 7 baffles. The linear speed of the belt was 72 feet per minute. Water was supplied to the belt at the rate of 245 gallons per minute. A total of 2400 pounds of chemically treated ore fines was fed to the belt at a rate of 24 long tons per hour. The results are recorded in the following table.

|            | Weights | B. P. L. | Recoveries | 65 |
|------------|---------|----------|------------|----|
|            | Percent | Percent  | Percent    |    |
| Heads..... | 100.0   | 36.28    | 100.0      |    |
| Concs..... | 52.2    | 66.63    | 90.0       |    |
| Tails..... | 47.8    | 3.06     | 4.0        |    |

*Example 3—(Cleaning test).*—The first half of the belt was equipped with type 5 baffles and the last half with types 6 and 7. The linear speed of the belt was 38 feet per minute. Water was supplied to the belt at the rate of 217 gallons per minute. Approximately 1200 pounds of roughing concentrates were fed to the belt at a rate of 15

75

long tons per hour. The results are recorded in the following table.

|            | Weights | B. P. L. | Recoveries |
|------------|---------|----------|------------|
|            | Percent | Percent  | Percent    |
| Heads..... | 100.0   | 60.64    | 100.0      |
| Concs..... | 70.6    | 74.88    | 87.2       |
| Middl..... | 29.4    | 26.88    | 12.8       |

*Example 4—(Cleaning test).*—The whole length of the belt was equipped with type 5 baffles. The linear speed of the belt was 72 feet per minute. Water was supplied to the belt at the rate of 285 gallons per minute. Approximately 1200 pounds of roughing concentrates were fed to the belt at a rate of approximately 30 tons per hour. The results are recorded in the following table.

|            | Weights | B. P. L. | Recoveries |
|------------|---------|----------|------------|
|            | Percent | Percent  | Percent    |
| Heads..... | 100.0   | 62.10    | 100.0      |
| Concs..... | 72.6    | 74.67    | 87.3       |
| Middl..... | 27.4    | 28.82    | 12.7       |

While we have shown and described the preferred embodiment of our invention, we do not desire to limit ourselves to the specific form illustrated, but may alter the construction and arrangement of parts as occasion requires without enlarging the scope of our invention or departing from the spirit thereof as contained in the appended claims.

We claim as our invention:

1. An ore concentrating machine comprising a belt apparatus having an ore receiving upper surface, means for driving said belt apparatus, a plurality of fixed baffles extending substantially throughout the length of the movable ore receiving upper surface and along the respective sides of the same, the baffles being angularly situated with relation to the belt apparatus to point in its direction of motion, said apparatus providing an unimpeded passageway along the belt between the baffles for the ore, and means for supplying ore and fluid to the apparatus.

2. An ore concentrating machine comprising a belt apparatus having a flat horizontal ore receiving upper belt surface, means for driving said belt apparatus, a plurality of stationary laterally located baffles in contact with the upper belt surface, said baffles substantially extending the length of the upper belt surface along its respective side portions and being situated at an inclination of from 20° to 45° with respect to a center line indicating the direction of motion of the belt, and means for supplying ore and fluid to the belt.

3. An ore concentrating machine comprising a belt apparatus having a flat horizontal ore receiving upper belt surface, means for driving said belt apparatus, a plurality of fixed baffles extending substantially throughout the length of the movable upper belt surface and along the respective sides of the same, said baffles being angularly situated at an inclination of from 20° to 45° with respect to a center line indicating the direction of motion of the belt, the portion of the apparatus between the respective side baffles being open to permit the direct passage of ore along the belt, and means for supplying ore and fluid to the belt.

4. An ore concentrating machine comprising a

belt apparatus having a flat horizontal ore receiving upper belt surface, means for driving said belt apparatus, a plurality of stationary baffles in contact with the movable upper belt surface and substantially extending throughout the length of the belt in rows along the respective side surfaces of the same, the baffles being angularly situated at an inclination of from 20° to 45° with respect to the center line indicating the direction of motion of the belt, said apparatus providing a direct passageway along the belt between the baffles for the ore, and means for supplying ore and fluid to the belt.

5. An ore concentrating machine comprising a belt apparatus having a flat ore receiving upper belt surface, means for driving said belt apparatus, a plurality of fixed perpendicular plate and horizontal rod baffles in contact with the movable upper belt surface, said baffles extending in rows along the respective sides of the upper belt surface and being angularly positioned to direct the ore toward the longitudinal center of the belt during its movement and means for supplying ore and fluid to the belt.

6. An ore concentrating machine comprising a belt apparatus, a plurality of stationary baffles situated along each side of the upper surface area of the belt apparatus, said baffles being angularly positioned to direct the ore away from the edge of the belt during its movement, means for driving said belt apparatus, and means for supplying ore and fluid to the same.

7. An ore concentrating machine comprising a belt apparatus having a flat ore receiving upper surface, means for driving said belt apparatus, a plurality of fixed baffles situated above the movable ore receiving surface, said baffles being arranged in rows along the respective sides of the belt surface to direct the ore moving upon the same toward its longitudinal center, and means for supplying ore and fluid to the apparatus.

8. In an ore concentrating machine, the combination of a belt apparatus having a transversely level ore receiving upper surface, a plurality of relatively closely spaced rigid baffles situated above the ore receiving surface of the belt, said baffles being located in parallel arrangement along substantially the entire side of the belt surface and being angularly positioned to point in direction of motion of the belt, the baffles extending partially across the width of the belt to provide an area adjacent the inwardly disposed ends of the same for the free passage of ore upon the belt, means for driving the belt apparatus, and means for supplying ore and fluid to the free passage area of the belt.

9. In an ore concentrating machine, the combination of a belt apparatus having a substantially flat ore receiving upper surface, a plurality of relatively closely spaced, angularly located, rigid baffles situated in a fixed position with relation to the upper surface of the belt, said baffles being located in substantially parallel arrangement along the entire side of the belt surface, the baffles extending partially across the width of the belt to provide an area adjacent the inwardly disposed ends of the same for the free passage of ore upon the belt, means for driving said belt apparatus, and means for supplying ore and fluid to the free passage area of the belt.